

Patented Nov. 29, 1927.

1,650,989

## UNITED STATES PATENT OFFICE.

PAUL KARRER, OF ZURICH, SWITZERLAND, ASSIGNOR TO CHEMICAL WORKS  
FORMERLY LANDOZ, OF BASEL, SWITZERLAND.

### PROCESS FOR THE PREPARATION OF COTTON FIBERS.

No Drawing. Application filed March 6, 1926, Serial No. 92,953, and in Germany March 11, 1925.

It has been found that cotton fibers, which are more or less esterified with toluene sulphonic, benzene sulphonic and naphthalene sulphonic groups or with aryl- and alkylsulphonic groups of any kind, can be altered by treating them with inorganic basic nitrogen compounds, for instance aminonia, hydrazine etc., so that the fibers are capable of being directly dyed with acid dyestuffs of 10. any kind.

The process can be performed by treating the above mentioned esterified cotton fibers with these substances, pure or dissolved in suitable solvents, which are not injurious to 15. the fibers, for example water, alcohol etc., or by treating the fibers in the cold with the above mentioned agents. Ammonia for instance can also be employed in form of gas.

The following example illustrates the invention without however limiting its scope, the parts being by weight.

10 parts of cotton, partially esterified by toluene sulphonic groups, are heated with

50 parts of a 25% watery ammonia solution for 6 hours in an autoclave at 100° C. The 25 duration of the heating can be prolonged or shortened.

The fibers thus treated can be dyed directly with acid dyestuffs such as tartrazine, orange II, sulphorhodamine and most 30 others.

What I claim is:

1. A process for the preparation of cotton fibers in view of their direct dyeing with acid dyestuffs, consisting in treating cotton 35 fibers which are partially esterified with an organic sulphonic group, with an inorganic basic nitrogen compound.

2. A process for the preparation of cotton fibers in view of their direct dyeing with 40 acid dyestuffs, consisting in treating cotton fibers which are partially esterified with an organic sulphonic group, with ammonia.

In witness whereof I have hereunto signed my name this 17th day of February, 1926.

PAUL KARRER.